

## UNITED STATES PATENT OFFICE

2,614,981

PROCESS FOR INHIBITING CORROSION IN  
OIL WELLS

Melba L. Lytle, Houston, Tex., assignor, by mesne assignments, to Standard Oil Development Company, Elizabeth, N. J., a corporation of Delaware

No Drawing. Application April 3, 1950,  
Serial No. 153,768

12 Claims. (Cl. 252—8.55)

1

The present invention is directed to a method for inhibiting the corrosiveness to corrodible metal surfaces of corrosive subsurface fluids containing carbon dioxide. More particularly, the invention relates to a method for inhibiting the corrosivity of petrolierous well fluids containing carbon dioxide to corrodible ferrous metal conduits and attendant equipment through which the fluids are flowed and processed.

In many oil fields and gas-condensate fields, the production of fluids from subsurface formations is accompanied by extremely severe corrosion of the conduits and attendant equipment which is contacted by the fluid mixture being produced. In many cases it is found that the fluid mixture is acidic in nature and contains substantial amounts of carbon dioxide, a portion of which dissolves in water present in the fluids to form carbonic acid. These fluids, including the carbon dioxide, originate in the subsurface formations. In some cases the corrosion occurs throughout the conduits and attendant equipment through which the fluids are flowed and processed while in other cases the corrosion is limited primarily to rather restricted areas of the conduit and is often particularly severe in that portion of the conduit adjacent the well head. If corrosion, whether intensive or extensive, is permitted to continue unabated, the conduit and attendant equipment will become sufficiently damaged to require replacement. Not only is the actual cost of such replacement high, but other factors may be involved which further increase costs. For example, it may be necessary to kill a high pressure well in order to make the necessary replacements. Furthermore, while replacements and repairs are being made, there is a loss in revenues due to having the well off production. Even of more importance than the high costs incurred as a result of corrosion, is the danger that a well will flow wild as a result of the failure of the conduit or equipment due to corrosion. Such a result may be catastrophic.

It is therefore the main object of the present invention to provide a method whereby corrosion of corrodible ferrous metal surfaces by corrosive well fluids containing carbon dioxide is substantially eliminated or inhibited.

In accordance with the present invention the corrosion to corrodible ferrous metal surfaces by corrosive well fluids including brine and carbon dioxide is eliminated or substantially reduced by incorporating in the corrosive fluids a corrosion inhibiting amount of a fatty derivative of an alkyl or an alkanol amine. This fatty derivative is prepared by reacting a fatty material selected from the class of fatty oils and fatty acids with an alkyl or alkanol amine at a temperature in the

2

range of 300° to 550° F. preferably in the presence of an alkaline reacting catalyst.

Fatty acids which may suitably be used as the fatty material in the aforementioned reaction include those fatty acids having at least 12 and no more than 26 carbon atoms per molecule. As examples of such acids, mention may be made of oleic, ricinoleic, linoleic, linolenic, licanic, eleostearic, arachidonic, clupanodonic, lauric, myristic, arachidic, stearic, palmitic, etc. The fatty oils which may be employed are those from which fatty acids having from 12 to 26 carbon atoms in the molecule can be derived. Fatty oils which have been found to produce especially effective agents include tung oil, China-wood oil, oiticica oil, chaulmoogra oil, cottonseed oil, menhaden oil, linseed oil, castor oil, and the like. It will be understood, of course, that mixtures of individual members of the aforementioned class of oils or mixtures of the individual members of the aforementioned class of acids or mixtures including both oils and acids may be employed as the fatty material from which the corrosion inhibiting agent of the present invention is produced.

Various alkyl and/or alkanol amines may suitably be employed in the aforementioned reaction to produce the corrosion inhibiting reaction product of the present invention. Examples of alkanol amines which may be employed include triethanol amine, di-n-propanol amine, di-isopropanol amine, tri-n-propanol amine, tri-isopropanol amine, di-n-butanol amine, di-isobutanol amine, tri-n-butanol amine, tri-isobutanol amine, tri-tert. butanol amine, etc. Examples of alkyl amines which may be employed include triethyl amine, di-n-propyl amine, di-isopropyl amine, di-n-butyl amine, di-isobutyl amine, di-tert. butyl amine, tri-n-propyl amine, tri-isopropyl amine, tri-n-butyl amine, tri-isobutyl amine, tri-tert. butyl amine, tri-amyl amine (and its isomeric forms), tri-hexyl amine (and its isomeric forms), etc. Rather than containing only alkanol or alkyl groups, the amines employed may contain both alkanol and alkyl groups. Examples of such alkyl-alkanol amines include di-ethyl, ethanol amine; ethyl, di-ethanol amine; ethyl, di-n-propanol amine; di-ethyl, n-propanol amine; ethyl, di-isopropanol amine; di-ethyl, isopropanol amine; n-propyl, di-ethanol amine; isopropyl, di-ethanol amine; di-n-propyl, ethanol amine; di-isopropyl, ethanol amine; ethyl, di-butanol amine; etc. While the amines employed preferably contain a total of between 6 and 18 carbon atoms in the alkyl and/or alkanol side chains, they may contain an even larger number of carbon atoms in the side chains. It will be understood, of course, that mixtures of the aforementioned

amines may suitably be employed. Polymers of these amines, such as the polymers of tri-ethanol amine, may also suitably be employed.

When the fatty derivatives of the present invention are prepared from a fatty oil, it is preferable that the fatty oil be present in the initial reaction mixture in a weight ratio of from about 1:1 to about 5:1 as compared to the alkyl or alkanol amine. When the fatty derivative is prepared from a fatty acid, the fatty acid is preferably present in the initial reaction mixture in a weight ratio of from about 0.5:1 to about 3:1 as compared to the amine.

The effectiveness as a corrosion inhibiting agent of the reaction product of fatty oils and/or fatty acids with alkyl amines and/or alkanol amines depends upon the temperature at which the reaction is conducted. If the reaction is conducted at a temperature below about 300° F., the resulting reaction product possesses little, if any, effectiveness as a corrosion inhibiting agent for gas-condensate well fluids containing carbon dioxide. On the other hand, if the reaction is conducted at a temperature in excess of about 550° F., the reaction product obtained tends to be of very high solidification point and of low solubility in the corrosive media. The reaction temperature selected will depend to some extent upon the particular fatty oil or acid employed and upon the particular amine employed. For example, when the corrosion inhibiting agent is prepared from triethanol amine and either tung oil, oiticica oil, chaulmoogra oil, or cottonseed oil in the presence of sodium hydroxide, a reaction temperature maintained for 2 to 4 hours in the range of 400° to 475° F. results in a product of especially desirable inhibition properties.

The extent of reaction, in addition to depending upon reaction temperature, also depends upon the time during which the reaction is permitted to continue. Ordinarily, an effective agent may be prepared when the reactants are maintained at a temperature in the aforementioned range for a period of time in the range of from 1/2 to 5 hours, although the preferred time is in the range of 1 1/2 to 4 hours.

As hereinbefore mentioned, an alkaline reacting catalyst, such as alkali metal hydroxides or carbonates, or mixtures thereof, is preferably employed. The fatty acids and amines will react to form the desired product without the aid of a catalyst; the fatty oils, however, require the use of a catalyst to accelerate the reaction between the oil and the amine. Examples of alkaline reacting catalysts are sodium hydroxide and sodium carbonate. The alkaline reacting catalyst concentrations ordinarily need not exceed about 3% by weight of the reactants although considerably lower concentrations may be successfully employed. For example, a concentration of 0.5% by weight of sodium hydroxide or sodium carbonate based upon the weight of the reactants has been found sufficient to promote the reaction. As a matter of fact, as little as about 0.05% of sodium hydroxide based upon the weight of the reactants has been found sufficient. Of course, mixtures of sodium hydroxide and sodium carbonate may be employed.

On completion of the reaction, the reaction product is allowed to cool and may be incorporated as such in the corrosive fluid to be treated or may be first dissolved in a suitable solvent such, for example, as an aromatic solvent or kerosene, and the solution incorporated in the corrosive fluid.

The amount of fatty derivatives of the present invention employed to inhibit the corrosion of ferrous metal surfaces by well fluid mixtures including moisture and carbon dioxide may be varied over a relatively wide range. However, it has been found that amounts within the range of 0.005% to 0.1% by volume of the fluid mixture give satisfactory results. Ordinarily, an amount within the range of 0.005% to 0.01% by volume will be sufficient.

When it is desired to protect from corrosion the conduit in the borehole as well as the attendant equipment, the fatty derivative or a solution thereof may be injected into the borehole adjacent the subsurface formation from which the corrosive fluid, including carbon dioxide, is produced. Alternatively, the fatty derivative may be introduced directly into the conduit. A still further method of introducing the fatty derivative into the fluids produced from the subsurface formation involves introducing the fatty derivative or a solution thereof into the annular space between the casing and the tubing. Another method of introducing the fatty derivative into the subsurface fluid consists of injecting the fatty derivative or a solution thereof into the subsurface reservoir through an adjacent well. Irrespective of the particular procedure employed in introducing the fatty derivatives into the fluids in the well, the fatty derivative suppresses the corrosivity of the fluids, thereby eliminating or reducing damage to the conduit through which the fluids are produced and to attendant equipment through which the fluids are flowed.

The following examples will illustrate the effectiveness of the corrosion inhibitors hereinbefore described in inhibiting the corrosivity of a corrosive condensate well fluid containing carbon dioxide to corrodible ferrous metal surfaces.

#### EXAMPLE I

40 parts by weight of triethanol amine, 52 parts by weight of tung oil, and 2 parts by weight of sodium hydroxide were heated together at 445° to 465° F. for a period of about 5 hours. In order to test the effectiveness of the reaction product thus formed, 0.001 volume per cent was added to a beaker containing 200 cc. of corrosive water from the gas-condensate field at Katy, Texas. This beaker, together with another beaker containing 200 cc. of water from the gas-condensate field at Katy, Texas, was placed in a desiccator. A mild carbon steel coupon was submerged in the water in each of the beakers. The desiccator was then evacuated and carbon dioxide was added to the desiccator to a pressure of 1 atmosphere. Each of the coupons was removed from the desiccator after 21 days' exposure under the aforementioned conditions and the extent of the corrosion of each coupon was determined by measuring the loss in weight of the coupons. The results of the tests are shown in the following table:

Table I

| Inhibitor                                                           | Cone. of Inhibitor Vol. Per cent | Corrosion Rate of Coupons In./Yr. | Percent Reduction Over Blank |
|---------------------------------------------------------------------|----------------------------------|-----------------------------------|------------------------------|
| None                                                                |                                  | 0.0077                            |                              |
| Reaction Product of Triethanolamine, Tung Oil, and Sodium Hydroxide | 0.01                             | 0.0009                            | 89                           |

## EXAMPLE II

35 grams of tung oil, 30 grams of triamylamine, and 2 grams of sodium hydroxide were heated together at a temperature of 392° to 432° F. for a period of 2 hours. The resulting reaction product, when cooled, solidified at a temperature of 244° F. The effectiveness of this reaction product as an inhibitor was tested in the laboratory by using a concentration of 0.01 weight per cent in a 50:50 mixture of brine and condensate saturated with carbon dioxide. The brine and condensate were obtained from the gas-condensate field located at Katy, Texas. 100 cc. of the aforementioned oil-brine mixture containing the inhibitor were placed in a sealed glass tube and a mild carbon steel coupon was suspended in the tube. The coupon was immersed in the brine-oil mixture 31 times per minute for a period of 14 days. The extent of the corrosion inhibition obtained was compared with results obtained when similar coupons were exposed under identical conditions to a carbon dioxide saturated 50:50 mixture of brine and condensate obtained from the Katy field, this last mentioned mixture containing no inhibitor. The results obtained are shown in Table II below:

Table II

| Inhibitor                                                        | Cone. of Inhibitor Wt. Percent | Corrosion Rate of Coupons In./Yr. | Percent Reduction Over Blank |
|------------------------------------------------------------------|--------------------------------|-----------------------------------|------------------------------|
| None                                                             | -----                          | 0.0054                            | -----                        |
| Reaction Product of Tung Oil, Triamylamine, and Sodium Hydroxide | 0.01                           | 0.0008                            | 89                           |

The foregoing examples demonstrate the effectiveness of the inhibiting agent of the present invention in substantially eliminating the corrosivity of condensate well fluids containing carbon dioxide to corrodible ferrous metal surfaces.

Having fully described the present invention, what I desire to claim as new and useful and to secure by Letters Patent is:

1. A method for reducing the corrosiveness to corrodible ferrous metal of a corrosive petroliferous well fluid including moisture and carbon dioxide which comprises introducing into said fluid a corrosion inhibiting amount of the reaction product of a fatty material selected from the group consisting of fatty acids having no less than 12 and no more than 26 carbon atoms per molecule and a fatty oil containing fatty acid radicals having no less than 12 and no more than 26 carbon atoms with an amine selected from the group consisting of alkyl and alkanol amines having a total of no less than 6 carbon atoms in the molecule, the reaction product being formed at a temperature in the range of 300° to 550° F. and in the presence of an alkaline reacting catalyst selected from the group consisting of alkali metal hydroxide and alkali metal carbonate, the weight ratio of fatty material to amine being in the range of 0.5:1 to about 5:1.

2. A method for reducing the corrosiveness to corrodible ferrous metal of a corrosive petroliferous well fluid including moisture and carbon dioxide which comprises introducing into said fluid a corrosion inhibiting amount of the reaction product of a fatty material selected from the group of fatty acids having no less than 12 and no more than 26 carbon atoms per molecule and a fatty oil containing fatty acid radicals

having no less than 12 and no more than 26 carbon atoms with an amine selected from the group consisting of alkyl and alkanol amines having a total of no less than 6 and no more than 18 carbon atoms per molecule, the reaction product being formed by heating the reactants for a period of from  $\frac{1}{2}$  to 5 hours at a temperature in the range of 300° to 550° F. in the presence of an alkaline reacting catalyst selected from the group consisting of alkali metal hydroxide and alkali metal carbonate, the weight ratio of fatty material to amine being in the range of 0.5:1 to about 5:1.

3. A method in accordance with claim 1 in which the reaction product is added to the corrosive fluid in an amount in the range of 0.005% to 0.1% by volume of the fluid.

4. A method in accordance with claim 2 in which the reaction product is added to the corrosive fluid in an amount in the range of 0.005% to 0.1% by volume of the fluid.

5. A method for reducing the corrosiveness to corrodible ferrous metal of a corrosive petroliferous well fluid including moisture and carbon dioxide which comprises introducing into said fluid a corrosion inhibiting amount of the reaction product formed by heating a mixture of tung oil and triethanol amine at a temperature in the range of 300° to 550° F. for a period of from  $\frac{1}{2}$  to 5 hours in the presence of an alkaline reacting catalyst selected from the group consisting of alkali metal hydroxide and alkali metal carbonate, the weight ratio of tung oil to triethanol amine being in the range of 1:1 to about 5:1.

6. A method in accordance with claim 5 in which said reaction product is added to the corrosive fluid in an amount in the range of 0.005% to 0.1% by volume of the fluid.

7. A method for reducing the corrosiveness to corrodible ferrous metal of a corrosive petroliferous well fluid including moisture and carbon dioxide which comprises introducing into said fluid a corrosion inhibiting amount of the reaction product formed by heating a mixture of tung oil and triamyl amine at a temperature in the range of 300° to 550° F. for a period of from  $\frac{1}{2}$  to 5 hours in the presence of an alkaline reacting catalyst selected from the group consisting of alkali metal hydroxide and alkali metal carbonate, the weight ratio of tung oil to triamyl amine being in the range of 1:1 to about 5:1.

8. A method in accordance with claim 7 in which the reaction product is added to the corrosive fluid in an amount in the range of 0.005% to 0.1% by volume of the fluid.

9. A method for reducing the corrosiveness to corrodible ferrous metal of a corrosive petroliferous well fluid including moisture and carbon dioxide which comprises introducing into said fluid a corrosion inhibiting amount of the reaction product formed by heating a mixture of cottonseed oil and triethanol amine at a temperature in the range of 300° to 550° F. for a period from  $\frac{1}{2}$  to 5 hours in the presence of an alkaline reacting catalyst selected from the group consisting of alkali metal hydroxide and alkali metal carbonate, the weight ratio of cottonseed oil to triethanol amine being in the range of 1:1 to about 5:1.

10. A method in accordance with claim 9 in which the reaction product is added to the corrosive fluid in an amount in the range of 0.005% to 0.1% by volume of the fluid.

11. A method for reducing the corrosiveness to corrodible ferrous metal of a corrosive petrolifer-

ous well fluid including moisture and carbon dioxide which comprises introducing into said fluid a corrosion inhibiting amount of the reaction product formed by heating a mixture of menhaden oil and triethanol amine at a temperature in the range of 300° to 550° F. for a period of from  $\frac{1}{2}$  to 5 hours in the presence of an alkaline reacting catalyst selected from the group consisting of alkali metal hydroxide and alkali metal carbonate, the weight ratio of menhaden oil to tri-ethanol amine being in the range of 1:1 to about 5:1.

12. A method in accordance with claim 11 in which the reaction product is added to the corrosive fluid in an amount in the range of 0.005% to 0.1% by volume of the fluid.

MELBA L. LYTHE.

#### REFERENCES CITED

The following references are of record in the file of this patent:

#### UNITED STATES PATENTS

| Number    | Name   | Date          |
|-----------|--------|---------------|
| 1,992,689 | Cox    | Feb. 26, 1935 |
| 2,366,013 | Duncan | Dec. 26, 1944 |
| 2,416,552 | Valko  | Feb. 25, 1947 |
| 2,460,259 | Kahler | Jan. 25, 1949 |
| 2,466,517 | Blair  | Apr. 5, 1949  |
| 2,470,965 | Woods  | May 25, 1949  |

#### OTHER REFERENCES

"Alkaterge"—Bulletin—Nov. 8, 1948—Commercial Solvents Corp.